

May 10, 1960

S. J. PORTER

2,935,948

ROCKET IGNITER PELLETS

Filed Feb. 14, 1958



Fig. 1



Fig. 2



Fig. 3

INVENTOR.

Samuel J. Porter

ECKHOFF & SLICK  
ATTORNEYS

By Robert A. Seay  
A MEMBER OF THE FIRM

1

2,935,948

## ROCKET IGNITER PELLETS

Samuel J. Porter, Scituate, Mass., assignor to American Potash & Chemical Corporation, a corporation of Delaware

Application February 14, 1958, Serial No. 715,421

2 Claims. (Cl. 102—70)

This invention relates in general to pellets used for the purpose of igniting the main propellant charge of a rocket device and more particularly to a coating for these rocket igniter pellets.

It is customary practice in the rocket ignition art to cause ignition of the main propellant charge by burning a quantity of readily ignitable pellets which are enclosed in the igniter prior to firing and ignited by squibs which are electrically actuated. After the pellets have become ignited, they are dispersed onto the grain surface of the rocket powder where they continue to burn and cause ignition of the rocket propellant. These pellets ordinarily consist of an ignition mixture such as potassium perchlorate, barium nitrate and zirconium nickel alloy with a small amount of a binder such as ethyl cellulose.

The pellets have reasonable mechanical strength, comparable to ordinary aspirin tablets, which they may resemble in size and shape. However, in practice it has been found that since these pellets are usually packed in the igniter, they tend, during handling and transportation, to rub and strike against each other with resultant attrition and breakage. The effect of this is that considerable dust formation occurs with consequent large increase in total surface of the ignition mixture. Thus, when the igniter functions, it very often explodes rather than burns in a controlled fashion since there is much more ignitable surface than originally intended. In other instances, if considerable breakage and dust formation results, enough packing down of the material around the squibs may occur that the fire from the squibs does not hit the igniter material as intended and non-ignition occurs.

Further, when the igniter pellets are formed into aspirin-sized cylinders, uniform size and weight is somewhat difficult to maintain and if the pellet compositions contain such abrasive metal powders as boron, there is considerable wear on the dies used.

Finally, since the pellets customarily are exposed to the atmosphere for a period of time before use, they may absorb a certain amount of moisture adversely affecting their operation.

It is therefore an object of this invention to provide means for eliminating the breakage and consequent increase in total surface area of the igniter pellets.

It is a further object of this invention to provide means for controlling the rate of burning of igniter pellets.

Still another object of this invention is to provide for greater quality control in the manufacture of igniter pellets and to provide a product which is moisture-resistant and which will withstand rough handling.

Broadly, it has been found that rocket ignition devices wherein a plurality of pellets are provided for dispersion onto a rocket grain surface after the ignition of the pellets may be improved substantially by providing a metallic jacket surrounding all or a large part of the exposed surface of the pellet, the metal being such a substance as aluminum, magnesium, titanium, zirconium or zirconium nickel alloys. Alloys of these five indi-

2

viduals are also suitable. The jacket must be consumed at the ignition temperature of the igniter pellet. The use of such a jacket or cup eliminates breakage and the formation of large quantities of powder and dust during handling of the pellets and thus insures the desired controlled burning.

The pellet may be entirely covered, one or two end surfaces being protected with very thin disks or sheets of metallic material of such a thickness that the application of heat by means of a squib of the type customarily employed in conjunction with igniters will cause destruction of the surface-protecting disk or sheet. Alternatively, a flat pellet surface may be left exposed, and the remaining surfaces and edges, which are normally more subject to chipping and breakage, covered with a suitable protective jacket or sleeve.

More particularly, it has been found that the igniter pellets ordinarily used in rocket igniters may be protected, moisture absorption controlled and improved quality control in terms of size and weight during manufacture obtained by the simple expedient of covering all or mostly all of the surfaces of the pellets with a thin jacket of metallic material, preferably aluminum, magnesium or titanium. If all surfaces of each pellet are to be protected and none left exposed, a surface of substantial size, such as one of the flat surfaces of an ordinary cylindrical pellet, should be covered with a metallic disk or sheet of a thickness no greater than about 0.005 inch and preferably 0.001 inch so that the heat supplied by the squib will cause destruction of this protective disk or sheet followed by ignition of the pellet. The jacket (exclusive of the disk or flat sheet protecting the single surface aforementioned) should be of a thickness of between about 0.005 and 0.010 inch. To serve effectively its primary purpose, that is, to protect the pellet from physical damage during handling, it need be of no greater thickness than this. Additional metal merely reduces the number of pellets which can be placed in a given volume.

As aforesaid, the jacket is composed of titanium, magnesium, aluminum, zirconium or alloys of these. Also suitable are the zirconium nickel alloys. Thus, on burning, the metallic jacket itself is consumed and contributes to the igniter performance. The metal used must be ignitable at or below the burning temperature of the igniter composition, and the disk fitted over one or both ends of the pellet must be capable of igniting at a temperature which can be produced by the squib-flame. Hence, the igniter composition has been modified to include in the formulation the metal represented by the jacket and, where the igniter composition ordinarily includes one of the metals listed above, as part of the admixture, the quantity thereof may be decreased by the amount of metal represented by the jacket. A preferred thickness for the jacket is about 0.010 inch and for the disk covering the flat surface of the pellet, about 0.001 to 0.002 inch.

In the drawings:

Figure 1 shows a standard cylindrical igniter pellet

jacketed on all sides except one flat surface;

Figure 2 shows a similar pellet provided with a thin aluminum protective disk on the upper surface thereof as well as the metal jacket on the other surfaces; and

Figure 3 is an isometric view of the rocket igniter assembly, partially cut away, showing the placement of the igniter-squib and the individual pellets surrounding the squib.

Considering now the drawings wherein like characters refer to like parts throughout, attention is directed to Figure 1 wherein the pellet, generally 10, is shown provided with the most elementary form of protection contemplated by this invention. A wedge has been removed

from the pellet to show the interior structure thereof. The ignited mix of the pellet, designated 12, is protected on its lower surface and on the peripheral circumferential walls thereof with a metallic cup 14. The upper surface is left entirely unprotected since it is the curved edges which have the greatest tendency to chip and break off. Of course, it is possible to leave both flat ends of the cylinder unprotected, the most essential feature being the protection of the more readily damaged curved walls of the pellet.

A modification of the invention is set forth in Figure 2. Metallic cup 16 covers the lower flat surface of the pellet and the peripheral circumferential walls, and is provided at the upper lip thereof with a flange 18 which serves to fasten in place the flat disk 20 provided for the protection of the upper surface of the pellet.

Figure 3 shows the entire igniter assembly, the base 22 having a squib initiator 24 of conventional structure positioned upright in the center thereof. Means 26 are provided for supplying an electrical impulse to the squib initiator 24. The assembly is provided with a cover basket 28 which seats upon the base 22 and serves to hold the individual pellets, in the fashion shown, clustered about the squib.

The structure of the igniter assembly is conventional and need not be described in greater detail here. Also, various pellet compositions are known to those skilled in the art, and it is to be understood that any of these may be used. That is, any of the known pellet compositions may be used provided that it is desired only to take advantage of the protection-affording features of the jacket. However, in the preferred embodiment of the invention, the composition used in combination with the jacket is one which ordinarily incorporates a metal or alloy as a portion of the customary formula. Thus, use of the jackets of this invention allows a substantial reduction in the quantity of metal used in the powder since the jacket itself is considered a portion of the formulation. The placement of the metal has been shifted from the interior of the pellet to the exterior thereof and hence it serves a twofold function simultaneously without adding any weight to the pellet. For example, a preferred embodiment of the invention involves an aluminum sleeve of 0.005 inch thickness filled with an igniter composition containing the following ingredients:

| Ingredient:            | Percent by weight |
|------------------------|-------------------|
| Potassium perchlorate  | 67.80             |
| Aluminum               | 4.78              |
| 50/50—zirconium/nickel | 13.62             |
| Boron                  | 9.45              |
| Ethyl cellulose        | 4.35              |
|                        | 100.00            |

The total width of the pellet including the sleeve is 0.290 inch and the thickness of the pellet is 0.125 inch.

The composition given above is to be contrasted with the corresponding original igniter composition prepared for use where an aluminum sleeve was lacking. Because of the absence of the aluminum in the form of the sleeve, the aluminum content of the igniter composition must be increased by the weight of the aluminum in the sleeve. Thus, the standard composition is as follows:

| Ingredient:            | Percent by weight |
|------------------------|-------------------|
| Potassium perchlorate  | 62.30             |
| Aluminum               | 12.50             |
| 50/50—zirconium/nickel | 12.50             |
| Boron                  | 8.70              |
| Ethyl cellulose        | 4.00              |
|                        | 100.00            |

A wide variety of igniter compositions are known to those in the field which contain various metals such as magnesium, aluminum, titanium, as well as zirconium

and zirconium-nickel alloys. For example, another very commonly used composition which may be modified readily by removing a portion of the zirconium-nickel alloy ordinarily contained in the composition and replacing it in the form of a protective sleeve, is the following composition:

| Ingredient:            | Percent by weight |
|------------------------|-------------------|
| Potassium perchlorate  | 30.00             |
| Barium nitrate         | 16.00             |
| Zirconium nickel alloy | 49.00             |
| Ethyl cellulose        | 5.00              |
|                        | 100.00            |

In a series of tests, igniter pellets (hereinafter designated I276) were loaded into thin aluminum cups of 0.010 inch thickness and one end of each pellet remained exposed. These pellets were loaded into an igniter basket of the type shown in the drawing and subjected to a regulation jumble test for thirty minutes. The composition of the pellets tested was:

| Ingredient:            | Percent by weight |
|------------------------|-------------------|
| Barium peroxide        | 84.00             |
| Toluidine, red pigment | 0.50              |
| Zinc stearate          | 1.00              |
| Magnesium powder       | 14.50             |
|                        | 100.00            |

These pellets emerged in better condition than did cellulose nitrate-treated pellets similarly tested or uncoated pellets also tested in this fashion.

In a further series of tests, these same pellets, following treatment as aforesaid, were ignited and the results compared. It was found that the pellets loaded into the aluminum cups burned with far less violence than did the other pellets. Details and results of each of these tests are set forth below.

The aforementioned igniter mix material for two of the tests was made into pellets 0.280 inch in diameter and approximately 0.125 inch high. In one test, the uncoated pellets were used. In a second test the pellets were coated with cellulose nitrate. This was applied by dipping the pellets twice in a 10% cellulose nitrate colloid in ethyl acetate. In the third test, the I276 was consolidated into regular aluminum relay cups with the load flush with the cup top. Approximately 85 grams of each type, i.e., pellets, coated pellets, and jacketed pellets, were loaded into an igniter basket with cotton batting in the bottom and the top sealed with a thin metal disk. The loaded baskets were then subjected to the jumble test for 30 minutes. The results were as follows:

| Type                 | Results                                            |
|----------------------|----------------------------------------------------|
| (1) Uncoated pellets | Nearly 100% broken.                                |
| (2) Coated pellets   | Slight erosion of pellet edges.                    |
| (3) Loaded cups      | Only a few minute scratches on the powder surface. |

Each of the above three loaded baskets was assembled to an igniter base containing squibs and sustainer mix. Each was then fired in the open with the following results:

| Type                 | Results                                                                                                                 |
|----------------------|-------------------------------------------------------------------------------------------------------------------------|
| (1) Uncoated pellets | Quite a severe initial blow which moved the whole unit approximately five feet. The sustainer burned for 12.5 seconds.  |
| (2) Coated pellets   | Quite a severe initial blow which moved the whole unit approximately three feet. The sustainer burned for 11.5 seconds. |
| (3) Loaded cups      | A mild initial blow which moved the whole unit approximately one foot. The sustainer burned for 10.5 seconds.           |

Additional tests have been conducted using titanium,

magnesium, zirconium and alloys of these as well as zirconium nickel alloys, and it has been found that thicknesses substantially identical to those set forth above as suitable for aluminum may be employed with satisfactory results.

It is seen, therefore, that by the use of a sleeve, cup or totally encompassing jacket, it is possible to avoid the objectionable chipping discussed above as well as securing a number of other advantages. In addition, when one of the metals suggested or an alloy thereof is used, such jacket will ignite and burn at a temperature less than the ignition temperature of the igniter composition, and hence the metal becomes a part of the igniter formula. However, it is necessary that the thickness of the metal sleeve and the disks used for covering the ends of the pellets be maintained to within the range of thicknesses set forth earlier if the desired consumption of the metal is to be achieved.

Obviously many modifications and variations of the invention as hereinbefore set forth may be made without departing from the spirit and scope thereof, and therefore only such limitations should be imposed as are indicated in the appended claims.

I claim:

1. In a rocket ignition device wherein a plurality of flat-ended cylindrical pellets consisting of an ignitable formulation containing at least one metal selected from the class consisting of aluminum, magnesium, and titanium, loosely contact one another in a container therefor, at least some of said pellets being juxtaposed to a 25 squib initiator therefor, the improvement comprising a sleeve of metal selected from the class consisting of aluminum, magnesium, titanium and alloys consisting solely of the foregoing metals encasing solely the circumferen- 30

tial walls of each of said pellets, the thickness of said metal being at least about 0.005 inch and no greater than about 0.010 inch, either end of each of said pellets remaining exposed, the metal of said sleeves serving as a portion of the total metal requirements of said pelleted formulation, and entering into the burning mechanism of said formulation.

2. In a rocket ignition device wherein a plurality of flat-ended, cylindrical pellets consisting of an ignitable formulation containing at least one metal selected from the class consisting of aluiminum, magnesium, and titanium, loosely contact one another in a container therefor, at least some of said pellets being juxtaposed to a 10 squib initiator therefor, the improvement comprising a cup of metal selected from the class consisting of aluminum, magnesium, titanium and alloys consisting solely of the foregoing metals encasing all but a single flat surface of each of said pellets, the thickness of said metal cup being at least about 0.005 inch and no greater than about 0.010 inch, one end of each of said pellets remaining exposed, the metal of said cups serving as a portion of the total metal requirements of said pelleted formulation.

References Cited in the file of this patent

UNITED STATES PATENTS

|           |           |       |               |
|-----------|-----------|-------|---------------|
| 1,036,176 | Bichel    | ----- | Aug. 20, 1912 |
| 2,072,671 | Foulke    | ----- | Mar. 2, 1937  |
| 2,124,201 | Lewis     | ----- | July 19, 1938 |
| 2,561,670 | Miller    | ----- | July 24, 1951 |
| 2,637,274 | Taylor    | ----- | May 5, 1953   |
| 2,685,837 | Sage      | ----- | Aug. 10, 1954 |
| 2,697,325 | Spaulding | ----- | Dec. 21, 1954 |